

# United States Patent

Chretien et al.

[15] 3,658,665

[45] Apr. 25, 1972

[54] **ELECTROLYTIC METHOD FOR PRODUCING A COLORED ANODIZED LAYER ON ALUMINUM AND ALLOYS OF ALUMINUM**

[72] Inventors: **Roland Chretien, Paris; Henri Richaud, Le Mans, both of France**

[73] Assignee: **Pechiney, Compagnie de Produits Chimiques et Electrometallurgiques, Paris, France**

[22] Filed: **Apr. 15, 1969**

[21] Appl. No.: **816,420**

**Related U.S. Application Data**

[63] Continuation-in-part of Ser. No. 495,708, Oct. 13, 1965, abandoned, Continuation-in-part of Ser. No. 651,971, July 10, 1967, abandoned.

[30] **Foreign Application Priority Data**

July 13, 1966 France ..... 69304

[52] U.S. Cl..... 204/58  
[51] Int. Cl. .... C23b 9/02  
[58] Field of Search..... 204/58, 35

[56] **References Cited**

**UNITED STATES PATENTS**

3,265,597 8/1966 Neunzig et al..... 204/58  
2,233,785 3/1941 Korpiun..... 204/58  
R25,566 4/1964 Deal et al..... 204/58

*Primary Examiner*—John H. Mack  
*Assistant Examiner*—R. L. Andrews  
*Attorney*—McDougall, Hersh, Scott & Ladd

[57] **ABSTRACT**

The invention is addressed to the coloring of aluminum and alloys of aluminum by anodization wherein the aluminum article is immersed as the anode in an electrolytic bath formulated of an aqueous solution of a naphthalene sulphonic acid or alkali metal salt thereof and sulphuric acid, with or without an aliphatic acid of carbon atoms.

**25 Claims, No Drawings**

**ELECTROLYTIC METHOD FOR PRODUCING A  
COLORED ANODIZED LAYER ON ALUMINUM AND  
ALLOYS OF ALUMINUM**

This application is a continuation-in-part of our copending applications Ser. No. 495,708, filed Oct. 13, 1965, and entitled **Method for Producing Colored Oxide Layers on Alloys of Aluminum by Anodic Oxidation and Composition**, and Ser. No. 651,971, filed July 10, 1967, and entitled **Method for Producing Colored Anodized Layer on Aluminum and Alloys of Aluminum** both now abandoned.

This invention relates to the production of colored aluminum oxide layers by electrolytic treatment of aluminum or alloys of aluminum and it relates to the formulation of the electrolytic bath and to products produced thereby.

To the present, colored layers have been produced on aluminum and alloys of aluminum by a two stage process in which a colorless oxide of aluminum is first formed on the surface by anodic oxidation in an electrolyte containing sulphuric acid. Thereafter the formed anodized layer of aluminum oxide is colored by the use of suitable colored pigments. From the architectural standpoint, the process described is insufficient by reason of the instability and non-uniformity of the formed colored layer.

Colored layers have also been formed on aluminum and alloys of aluminum in a one stage process wherein use is made of an electrolytic bath formulated to contain an organic acid or salt thereof, when certain conditions are maintained during the electrolysis. For example, additions of oxalic acid to the electrolyte and the use of high current densities will operate to produce an oxide layer having a gold tint when use is made of direct current and a brownish layer when use is made of alternating current. The color intensity is sufficient only if very thick layers on the order of 50 to 600 microns are produced and the layers are generally non-uniform in color.

Electrolytes formulated to contain other organic compounds have also been proposed, such as sulphosalicylic acid in German Pat. No. 657,902, but the colors obtained are weak unless layers of substantial thickness are produced.

It is an object of this invention to produce and to provide a method for producing relatively thin layers of high and uniform color intensity on aluminum and alloys of aluminum by electrolytic treatment and it is a related object to produce a new and improved electrolyte for use in the practice of same.

It has been found, in accordance with the practice of this invention, that a coloration of high color intensity and good uniformity can be obtained on the surface of aluminum and alloys of aluminum by the use of an electrolyte formulated to contain a mixture of sulphuric acid and 2-naphthol-6, 8-disulphonic acid (G acid), 2-naphthol-3, 6-disulphonic acid (H acid), 1, 8-dihydroxynaphthalene-3, 6-disulphonic acid (chromotropic acid) or 1-naphthol-8-amino-3, 6-disulphonic acid. Instead of making use of one or more of the described free sulphonic acids, use can be made of the ammonium, alkali metal or other water soluble salts thereof. Anodic treatment in the electrolyte will give a fine gold color to aluminum or a color ranging from bronze, beige, grey or chestnut to alloys of aluminum, depending somewhat upon the composition of the alloy.

In practice, the composition and conditions can be varied over fairly wide limits. The naphthalene sulphonic acid component can be employed in solution in the aqueous electrolytic bath in an amount within the range of 1-200 grams per liter and preferably within the range of 20-200 grams per liter. The amount of sulphuric acid should not exceed 50 grams per liter and it is preferred to formulate the aqueous electrolytic bath with an amount of sulphuric acid within the range of 3-10 grams per liter. Gold layers of greater harness can be obtained when the amount of sulphuric acid is maintained within the range of 5-10 grams per liter.

The anodic oxidation of the aluminum or alloy of aluminum in the electrolytic bath can be carried out with direct current or with alternating current or by superimposing an alternating current on a direct current, in a system generally referred to as pulsating current. Current densities can be used ranging from

1 to 10 A/dm<sup>2</sup> and preferably within the range of 1.5 to 4.5 A/dm<sup>2</sup>. The temperature of the electrolyte can be varied during operation within the range of 0° to 70° C. but it is preferred to make use of a temperature within the range of 15° to 30° C.

Under these conditions, a suitable coating can be obtained within a time ranging from 1 to 120 minutes depending somewhat upon the thickness of the coating desired and the current density. During the electrolytic treatment, it is desirable to maintain the electrolytic bath in a state of agitation either by the use of mechanical stirring means or by the use of gaseous streams.

The electrolytic treatment should be preceded by the usual steps for preparation of the sheet or shaped metal product such as by the processing steps of polishing, degreasing and pickling, and the electrolytic treatment should be followed by the usual procedures of rinsing, sealing and perhaps brightening.

The resulting product will have a layer of uniform color over the entire exposed surface and in which a color of sufficient intensity will be available in a layer having a thickness in the order of about 10 microns but in which the intensity of color can be further increased in proportion to the increased thickness of the color layer which may be as great as 30 microns or more.

The following examples are given by way of illustration, but not by way of limitation of our invention:

**EXAMPLE 1**

In this series of examples the sheets or shaped elements of aluminum or alloys of aluminum, as indicated in the following table, were polished mechanically, degreased with trichlorethylene, and pickled by soaking for 10 minutes in a 20° to 25° C. bath containing, per liter, 300 cc. of nitric acid, 10 grams of sodium fluoride and 1 cc. of a surface active agent such as an alkyl sulphonate, commercially known as CELANOL A. After rinsing, the elements were immersed in the electrolyte in the form of an aqueous solution containing 5 grams of sulphuric acid per liter and  $n$  grams of chromotropic acid per liter in which  $n = 5, 20$  and 100 grams. The current density was kept constant at the beginning at 2.5 A/dm<sup>2</sup> while the voltage at the terminals was progressively raised to 60 volts and thereafter a constant voltage of 60 volts was employed. The temperature was maintained at 20° C. In each case, the operation was carried out on three identical samples in which the first was withdrawn after 20 minutes, the second after 30 minutes, and the last after 45 minutes of electrolysis with the result that an average thickness of an oxide layer of 5 to 8 microns was produced on the first sample, 12 to 15 microns on the second sample, and 20 to 30 microns on the third sample.

The following table indicates the color which is obtained in which the colors differ according to the composition of the metal that is treated:

**TABLE I**

|       | Alloy     | Color              |
|-------|-----------|--------------------|
| 60    | Al 99.99% | pale gold          |
|       | Al 99.5%  | greyish beige      |
| A-GS  | Si 0.4%   |                    |
|       | Mg 0.47%  | bronze             |
| A-SG  | Si 1.1%   | bronze-grey        |
|       | Mg 1.0%   |                    |
| A-G3  | Mg 3%     | brown              |
| A-Z4G | Zn 3%     |                    |
|       | Mg 2%     | chestnut-black     |
| 65    | A-S5G     | grey-black         |
|       | Si 5%     |                    |
|       | Mg 0.5%   |                    |
| A-U4G | Cu 4%     |                    |
|       | Mg 0.5%   | grey-reddish brown |

The color of all of the samples was very uniform and the intensity of color increased in proportion to the increased thickness of the oxide layer. Very little difference is found to exist between the results when the content of chromotropic acid in the bath is varied in the amounts of 5, 20 and 100 grams per liter. This is an important factor because it becomes

superfluous to maintain a constant analysis of the composition of the bath for controlling the content of chromotropic acid and it also favors the ability to produce uniform results from piece to piece.

#### EXAMPLE 2

Sheets of aluminum alloy containing 3 percent magnesium, previously degreased with trichlorethylene and then cleaned for 10 minutes at 10° to 25° C. in a bath containing, per liter, 300 cc. of nitric acid, 10 grams of sodium fluoride and 1 cc. of alkyl sulphonate, followed by rinsing, are anodized in an aqueous bath containing the following ingredients and under the following conditions:

|                   |                     |
|-------------------|---------------------|
| chromotropic acid | 100 grams per liter |
| sulphuric acid    | 2 grams per liter   |

The electrolysis was operated at 2.5 A/dm<sup>2</sup> up to 60 volts and then with a substantially constant voltage of 60 volts and at a temperature of 22° C. After anodization for a period of 30 minutes, a deep brown oxide layer having a thickness of 20 microns was obtained.

#### EXAMPLE 3

Sheets of the same alloy as in Example 2 were subjected to the same surface preparation. They were then anodized in an aqueous bath containing 100 grams per liter of chromotropic acid and 20 grams per liter of sulphuric acid and operated at 2.5 A/dm<sup>2</sup> up to 60 volts and then under constant voltage of 60 volts at a temperature of 22° C. After anodizing for 30 minutes, a light brown layer having a thickness of 22 microns was obtained.

#### EXAMPLE 4

Sheets of the same alloy as in Example 2 were subjected to the same surface preparation and then were anodized in an aqueous bath containing 50 grams per liter of G acid and 7 grams per liter of sulphuric acid and operated at 4 A/dm<sup>2</sup> up to 60 volts and then at a constant voltage of 60 volts with a bath temperature at 20° C. After anodizing for 15 minutes, a deep brown oxide layer of 15 microns was obtained.

#### EXAMPLE 5

Shaped elements of aluminum alloy containing 1.10 percent by weight silicon, 1.00 percent by weight magnesium and 0.44 percent by weight manganese, the remainder aluminum, were subjected to the same surface treatment as in Example 2 and then anodized in an aqueous bath containing 100 grams per liter of chromotropic acid and 7 grams per liter of sulphuric acid and operated at 2.5 A/dm<sup>2</sup> up to 60 volts and then at a constant voltage of 60 volts, and at a temperature of 22° C. After anodizing for 30 minutes, a black oxide layer of 12 microns in thickness was developed.

#### EXAMPLE 6

Shaped elements formed of an aluminum alloy containing 0.40 percent by weight of silicon and 0.47 percent by weight of magnesium, the remainder aluminum, were subjected to the same surface preparation as in Example 2 and then anodized in an aqueous bath containing 40 grams per liter of H Acid and 9 grams per liter of sulphuric acid and operated at 3 A/dm<sup>2</sup> up to 60 volts and thereafter at a constant voltage of 60 volts with a temperature of 20° C. After 20 minutes, there was obtained a bronze colored oxide layer of 15 microns in thickness.

Bath composition of the types described find excellent use when it is desired to produce aluminum and alloys of aluminum having deeply colored shades on the surfaces thereof. Lighter shades can be produced by modification to raise both temperature or to reduce current density.

It has been found that the lighter shades obtained by temperature rise and/or reduction in current density can be markedly improved, at least from the standpoint of color uniformity, when the electrolytic bath is modified to include a third component in the form of an aliphatic acid having no more than five carbon atoms, such as a saturated mono-carboxylic acid, saturated dicarboxylic acid, or ethylenically unsaturated dicarboxylic acid, such as acetic acid, propionic acid, oxalic acid, succinic acid, maleic acid, itaconic acid and citraconic acid.

Such mixtures of naphthalene sulphonic acid, aliphatic acid and sulphuric acid enables the electrolytic treatment to be carried out at lower voltage and it enables the naphthalene sulphonic acid to be used in lower concentrations in the bath.

The amount of aliphatic acid use will depend somewhat on the nature of the acid and the effect desired to be secured but, in general, it is desired to make use of an electrolytic bath in which the aliphatic acid is present in an amount within the range of 10-100 grams per liter. The amount of naphthalene sulphonic acid can be reduced to less than 100 grams per liter and preferably within the range of 50-100 grams per liter or up to saturated solution when use is made of a naphthalene sulphonic acid containing an amino group.

Generally colored oxide layers having a thickness within the range of 10-30 microns should be produced. The colored layer that is formed is characterized by good hardness and excellent light and weather resistance.

The following examples are given by way of illustration, but not by way of limitation, of the further practice of this invention:

#### EXAMPLE 7

35 An aluminum alloy containing about 0.6 percent by weight of silicon and 0.7 percent by weight of magnesium is anodized in an aqueous bath containing in solution:

|    |                   |         |
|----|-------------------|---------|
| 40 | chromotropic acid | 50 g/l  |
|    | oxalic acid       | 10 g/l  |
|    | sulphuric acid    | 3.5 g/l |

45 Five tests were carried out with different current densities as set forth in the following table:

TABLE II

| No. of test | current density 1 a/dm <sup>2</sup> | temper-ature 20°C | dura-tion 60 mn | thickness of layer 15.5 μ | coloring      |
|-------------|-------------------------------------|-------------------|-----------------|---------------------------|---------------|
| 50          | 1                                   |                   |                 |                           | light         |
|             | 2                                   | 1.5 "             | 35 "            | 15 "                      | bronze        |
|             | 3                                   | 1.5 "             | 20°C            | 21 "                      | light bronze  |
|             | 4                                   | 1.8 "             | 20°C            | 19.5 "                    | medium bronze |
|             | 5                                   | 2.5 "             | 20°C            | 20 "                      | deep bronze   |

60 The aluminum oxide layer is hard, the color is very uniform and has excellent resistance to ultraviolet rays.

#### EXAMPLE 8

65 A sheet of commercial aluminum (99.5 percent Al) is anodized in an aqueous bath containing in solution:

|    |                   |         |
|----|-------------------|---------|
| 70 | chromotropic acid | 50 g/l  |
|    | acetic acid       | 100 g/l |
|    | sulphuric acid    | 7 g/l   |

75 The anodizing is carried out at 30° C. with a current density of 1.5 a/dm<sup>2</sup>. After 30 minutes, an oxide layer is obtained having a thickness of 15 microns and a light bronze color. The shade is very uniform and resistant to ultraviolet rays.

## EXAMPLE 9

Shaped elements of aluminum alloy having a composition the same as that in Example 7 are anodized for 30 minutes at 25° C. with a current density of 1.5 a/dm<sup>2</sup> in a bath containing chromotropic acid, maleic acid and sulphuric acid. Several tests were carried out in which the proportions of acids were varied as set forth in the following table:

TABLE III

| No. of test | Composition of bath                                     | Electrolysis on commence-<br>ment        | voltage<br>on completion | Color<br>of the layer       |
|-------------|---------------------------------------------------------|------------------------------------------|--------------------------|-----------------------------|
| 1           | chromotropic 100 g/l<br>maleic 50 "<br>sulphuric 3.5 "  | 41 V                                     | 50 V                     | medium<br>bronze            |
| 2           | chromotropic 100 g/l<br>maleic 75 "<br>sulphuric 3.5 "  | 40.5                                     | 50                       | bronze<br>lighter<br>than 1 |
| 3           | chromotropic 100 g/l<br>maleic 100 "<br>sulphuric 3.5 " | 40.5                                     | 52                       | bronze<br>lighter<br>than 2 |
| 4           | chromotropic 25 g/l<br>maleic 100 "<br>sulphuric 3.5 "  | no anodization<br>corrosion of the metal |                          |                             |
| 5           | chromotropic 50 g/l<br>maleic 100 "<br>sulphuric 3.5 "  | 42.5                                     | 48.5                     | deep<br>bronze              |
| 6           | chromotropic 50 g/l<br>maleic 100 "<br>sulphuric 7 "    | 34.5                                     | 42.5                     | light<br>bronze             |

It will be seen that with a bath containing 100 grams of chromotropic acid and 3.5 grams of sulphuric acid per liter, the increase in maleic acid content lightens the shade slightly but does not alter the electrolysis voltage necessary for maintaining the current density at 1.5 a/dm<sup>2</sup>.

The presence of maleic acid in the amount of 100 g/l permits the amount of chromotropic acid in the bath to be reduced to about 50 g/l. A content of sulphuric acid of the order of 7 g/l is preferred for reducing the electrolysis voltage.

## EXAMPLE 10

This example is intended to show the extent of the range of colors which can be obtained on aluminum or on alloys of aluminum with a bath of given composition merely by varying the current density and temperature. The aqueous bath was formulated of the following in solution:

|                   |         |
|-------------------|---------|
| chromotropic acid | 50 g/l  |
| maleic acid       | 100 g/l |
| sulphuric acid    | 7 g/l   |

TABLE IV

| Nature of metal        | current<br>density    | temper-<br>ature °C. | duration<br>min. | electrolysis voltage |                    |      | thick-<br>ness of<br>the layer | color |
|------------------------|-----------------------|----------------------|------------------|----------------------|--------------------|------|--------------------------------|-------|
|                        |                       |                      |                  | on com-<br>mencement | on com-<br>pletion |      |                                |       |
| 99.5% aluminum sheets. | 1.5 a/dm <sup>2</sup> | 30°                  | 40               | 33.5 V               | 36 V               | 18 μ | very<br>light                  |       |
|                        | 2.5                   | 25°                  | 20               | 37.5                 | 43                 | 16 μ | medium                         |       |
|                        | < 2.5 "               | 25°                  | 30               | 42.5                 | 48.5               | 15 μ | deep                           |       |
| Al shaped elements     | 1.5                   | 30°                  | 40               | 35                   | 40.5               | 16 μ | very                           |       |
| Si 0.6%                | 2                     | 25°                  | 20               | 34.5                 | 42.5               | 13 μ | light                          |       |
| Mg 0.7%                | 2.5                   | 20°                  | 30               | 37                   | 42.5               | 17 μ | medium                         |       |
| AAI sheets             | 2.5                   | 20°                  | 45               | 38                   | 60                 | 25 μ | black                          |       |
| Mg 0.5%                |                       |                      |                  |                      |                    |      |                                |       |
| Mn 0.5%                |                       |                      |                  |                      |                    |      |                                |       |
| Al shaped elements     |                       |                      |                  |                      |                    |      |                                |       |
| Si 1%                  | 2.5                   | 20°                  | 45               | 40                   | 60                 | 20 μ | black                          |       |
| Mg 0.5%                |                       |                      |                  |                      |                    |      |                                |       |
| Mn 0.5%                |                       |                      |                  |                      |                    |      |                                |       |

It will be apparent that, with the same bath composition, it is possible to obtain, on aluminum or on aluminum-magnesium-silicon alloys, shades which extend from very light bronze to deep bronze and that with aluminum-manganese-magnesium or aluminum-silicon-manganese-magnesium alloys, it is possible to obtain black shades.

## EXAMPLE 11

5 A shaped element of aluminum alloy containing 1 percent silicon, 0.5 percent magnesium and 0.5 percent manganese (by weight) is anodized in a bath formed of an aqueous solution of:

|    |                                                          |         |
|----|----------------------------------------------------------|---------|
| 10 | 1-naphthol-8-amino-3, 6-sulphonic acid (monosodium salt) | 25 g/l  |
|    | acetic acid                                              | 80 cc/l |
|    | sulphuric acid                                           | 5 g/l   |

15 Anodization was carried out with a current density of 2.5 a/dm<sup>2</sup> at 20° C. for 45 minutes. A black oxide layer of uniform appearance, having a thickness of 20 microns, is obtained.

## EXAMPLE 12

20 A shaped element of aluminum-magnesium-silicon alloy containing about 0.5 percent silicon and 0.5 percent magnesium (by weight) is anodized in a bath formed of an aqueous solution of:

|    |                                        |         |
|----|----------------------------------------|---------|
| 25 | 1-naphthol-8-amino-3, 6-sulphonic acid | 10 g/l  |
|    | propionic acid                         | 100 g/l |
|    | sulphuric acid                         | 6 g/l   |

30 The anodization is carried out at 20° C. with a current density of 2.5 a/dm<sup>2</sup>. After 30 minutes, a bronze colored layer of 20 microns is obtained. The shade is very uniform and it resists ultraviolet rays.

## EXAMPLE 13

35 A shaped element of aluminum-magnesium-silicon alloy containing 0.5 percent silicon and 0.5 percent magnesium (by weight) is anodized in a bath formed of an aqueous solution of:

|    |                                  |        |
|----|----------------------------------|--------|
| 40 | 2-naphthol-6, 8-disulphonic acid | 60 g/l |
|    | oxalic acid                      | 50 g/l |
|    | sulphuric acid                   | 3 g/l  |

45 The anodization is carried out at 25° C. with a current density of 1.5 a/dm<sup>2</sup>. After 45 minutes, a light bronze colored layer of 18 microns is obtained. The shade is very uniform and resistant to ultraviolet rays.

## EXAMPLE 14

50 Shaped elements of aluminum-magnesium-silicon alloy having the composition of Example 7 are anodized in an aqueous

bath containing:

|                                                     |         |
|-----------------------------------------------------|---------|
| 2-naphthol-6, 8-disulphonic acid (dipotassium salt) | 50 g/l  |
| oxalic acid                                         | 50 g/l  |
| sulphuric acid                                      | 3.5 g/l |

Anodization is carried out with a current density of 2.5 a/dm<sup>2</sup> at 25° C. for 40 minutes. A layer having a thickness of 25 microns is obtained with a medium bronze color. The shade is uniform in appearance and resistant to ultraviolet rays.

#### EXAMPLE 15

A commercial aluminum sheet (99.2 percent aluminum) is anodized in a bath formed of an aqueous solution of:

|                                             |         |
|---------------------------------------------|---------|
| 2-hydroxynaphthalene-3, 6-di-sulphonic acid | 50 g/l  |
| acetic acid                                 | 100 g/l |
| sulphuric acid                              | 7 g/l   |

The anodization is carried out at 20° C. with a current density of 2.5 a/dm<sup>2</sup>. After 30 minutes, a bronze colored layer having a thickness of 20 microns is obtained. The shade is uniform and resistant to ultraviolet rays.

#### EXAMPLE 16

A shaped element of aluminum-silicon-magnesium-manganese alloy containing about 1 percent silicon, 0.5 percent magnesium and 1 percent manganese (by weight) is anodized in a bath containing an aqueous solution of:

|                   |        |
|-------------------|--------|
| chromotropic acid | 50 g/l |
| succinic acid     | 65 g/l |
| sulphuric acid    | 5 g/l  |

The anodization is carried out at 20° C. with a current density of 2.5 a/dm<sup>2</sup> for 45 minutes. An anodized layer having a thickness of 25 microns is obtained which is black in color. The shade is very uniform and resistant to ultraviolet rays.

#### EXAMPLE 17

Sheets of an alloy consisting of aluminum with 3 percent magnesium are anodized in an aqueous bath containing:

|                   |         |
|-------------------|---------|
| chromotropic acid | 50 g/l  |
| citraconic acid   | 100 g/l |
| sulphuric acid    | 7 g/l   |

Anodization is carried out for 30 minutes at a voltage of 40 volts. A uniform brown anodized layer is obtained which is resistant to ultraviolet rays.

It will be understood that changes may be made in the details of formulation and conditions for anodization without departing from the spirit of the invention, especially as defined in the following claims.

We claim:

1. In a process for producing a colored layer on aluminum and alloys of aluminum by anodic oxidation in an electrolytic bath, the steps of mounting the aluminum article as an anode in the electrolytic bath formulated of an aqueous solution containing as essential ingredients the combination of sulphuric acid and a compound selected from the group consisting of 2-naphthol-6, 8-disulphonic acid, 2-naphthol-3, 6-disulphonic acid, 1, 8-dihydroxynaphthalene-3, 6-disulphonic acid and 1-naphthol-8-amino-3, 6-disulphonic acid, and water soluble salts thereof in which the sulphuric acid is present in an amount within the range of 1-200 grams per liter while the disulphonic acid derivative is present in an amount within the range of 1-200 grams per liter, and passing current between the electrodes through the bath.

2. A process as claimed in claim 1 in which the sulphuric acid is present in an amount up to 50 grams per liter.

3. A process as claimed in claim 1 in which the sulphuric acid is present in an amount from 3-10 grams per liter.

4. A process as claimed in claim 1 in which the disulphonic acid component is present within a range of 1-20 grams per liter.

5. The process as claimed in claim 1 which includes a step in maintaining the bath at a temperature within the range of 0° to 70° C during electrolysis.

6. The process as claimed in claim 1 which includes a step in maintaining the bath at a temperature within the range of 15°-30 C during electrolysis.

7. A process as claimed in claim 1 in which the current that is passed between the electrodes through the bath is direct current.

8. A process as claimed in claim 1 in which the current that is passed between the electrodes through the bath is alternating current.

10. 9. A process as claimed in claim 1 in which the current that is passed between the electrodes through the bath is pulsating current.

10. A process as claimed in claim 1 in which the current is passed at a current density of 1-10 A/dm<sup>2</sup>.

15. 11. A process as claimed in claim 1 in which the current is passed at a current density of 1.4 to 4.5 A/dm<sup>2</sup>.

12. An electrolytic bath for coloring aluminum and alloys of aluminum by anodization comprising an aqueous solution containing the combination of a naphthalene sulphonic acid selected from the group consisting of 2-naphthol-6, 8-disulphonic acid, 2-naphthol-3, 6-disulphonic acid, 1,8-dihydroxynaphthalene-3, 6-disulphonic acid and 1-naphthol-8-amino-3, 6-disulphonic acid, an aliphatic acid of less than five carbon atoms and sulphuric acid.

13. An electrolytic bath as claimed in claim 12 in which the naphthalene sulphonic acid or alkali metal salt is present in an amount within the range of 10 to 200 grams per liter.

14. An electrolytic bath as claimed in claim 12 in which the naphthalene sulphonic acid or alkali metal salt is present in an amount within the range of 50 to 100 grams per liter.

15. An electrolytic bath as claimed in claim 12 in which the naphthalene sulphonic acid or salt contains an amine group, and is present in the bath in an amount to saturate the solution.

16. An electrolytic bath as claimed in claim 12 in which the aliphatic acid is present in an amount within the range of 10 to 100 grams per liter.

17. An electrolytic bath as claimed in claim 12 in which the sulphuric acid is present in an amount within the range of 3 to 10 grams per liter.

18. An electrolytic bath as claimed in claim 12 in which the naphthalene sulphonic acid or its alkali metal salt is present in an amount within the range of 10 to 200 grams per liter, the aliphatic acid is present in an amount within the range of 10 to 100 grams per liter and the sulphuric acid is present in an amount within the range of 3 to 10 grams per liter.

19. An electrolytic bath as claimed in claim 12 in which the aliphatic acid is selected from the group consisting of saturated monocarboxylic acids, saturated dicarboxylic acids and ethylenically unsaturated dicarboxylic acids.

20. An electrolytic bath as claimed in claim 12 in which the aliphatic acid is selected from the group consisting of acetic acid, propionic acid, oxalic acid, succinic acid, maleic acid, itaconic acid and citraconic acid.

21. In the method of coloring aluminum and alloys of aluminum by anodizing, the step of immersing the aluminum or alloy of aluminum in an electrolytic bath as claimed in claim 12, as one electrode, providing another electrode in the bath and passing an electric current through the bath between said electrodes.

22. The method as claimed in claim 21 which includes the step of degreasing the aluminum base alloy before anodization.

23. The method as claimed in claim 21 which includes the step of sealing the anodized surface with an boiling aqueous solution of an organo metallic salt.

24. The method as claimed in claim 23 in which the salt dissolved in the sealing solution is nickel acetate present in the solution in an amount within the range of 0.5 to 1 gram per liter.

25. The method as claimed in claim 21 in which a color ranging from light to deep bronze is produced on aluminum and on aluminum-magnesium-silicon alloys and a black color is produced on aluminum-silicon-magnesium-manganese and aluminum-magnesium-manganese alloys.